

H. HESS.

METHOD OF CASTING.

APPLICATION FILED JUNE 18, 1913.

1,131,697.

Patented Mar. 16, 1915.



Fig. 1.



Fig. 2.

Fig. 3.

Fig. 4.

Witnesses:

H. R. Manning  
A. A. Robins

Inventor  
Henry Hess  
By his Attorney  
Rosen, Kennedy & Campbell

# UNITED STATES PATENT OFFICE.

HENRY HESS, OF PHILADELPHIA, PENNSYLVANIA.

## METHOD OF CASTING.

1,131,697.

Specification of Letters Patent. Patented Mar. 16, 1915.

Application filed June 18, 1913. Serial No. 774,832.

To all whom it may concern:

Be it known that I, HENRY HESS, a citizen of the United States, residing at Philadelphia, in the county of Philadelphia and State of Pennsylvania, have invented certain new and useful Improvements in Methods of Casting, of which the following is a specification, reference being had thereto in the accompanying drawing.

10 This invention relates to the production of cast objects such as ingots and the like, the object of the invention being to produce castings which will be sound and free from "pipes," shrinkage cavities, and like 15 defects so common with ingots as ordinarily produced; and the invention consists of an improved method of casting, in which the body of molten metal to form the casting or ingot, is subjected to a rotary motion, and 20 during its rotation, additional molten metal is supplied to the body in such manner as to prevent the formation of shrinkage cavities and like defects in the solidifying metal, and produce a sound casting solid throughout.

25 In the accompanying drawings I have represented, by way of example, a form of apparatus suitable for carrying my improved method into effect, but it will be manifest that other forms of apparatus may 30 be employed for this purpose, the present invention residing in the method of procedure without regard to the particular form of apparatus employed. Further it will be understood that my invention is not 35 limited to any particular mode or manner of treatment or manipulation of the molten metal, or sequence of steps in its treatment, except in so far as such limitations are specified in the claims.

40 In the accompanying drawings: Figure 1 is a vertical sectional elevation of a casting apparatus suitable for carrying my method into effect. Figs. 2, 3 and 4 are sectional elevations of the upper end of the mold 45 illustrating the different steps of the method.

In carrying my invention into effect in the preferred manner, I partially fill a mold with molten metal, and rotate the same 50 about an upright axis, and while rotating, I introduce additional molten metal into the mold until the mold is completely filled. This operation may be carried out by the apparatus shown in Fig. 1 in which an upper 55 right mold 1 is shown provided with a cover 2 containing a central pouring spout 3.

This mold is supported fixedly on a rotary table or support 4 so as to be rotatable with it, and the table is fixed to the upper end of a spindle 5 mounted in bearings in a frame 60 6, and rotated by intermeshing bevel gears 7 and 8 on the spindle and on the horizontal shaft 9 respectively. The shaft is provided with a driving pulley 10 adapted to be driven from any suitable source of power. 65

In the use of the apparatus in casting an ingot for instance, in accordance with my invention, the molten metal is poured into the spout 3 of the mold cover and the mold is rapidly rotated by the driving mechanism described. The metal partially filling the mold, will be caused by centrifugal force to rise at its sides in the mold as at 11 Fig. 2, thereby forming a central hollow or space 12 extending some distance down into 75 the body of metal. The pouring of the metal through the spout being continued, the added metal will flow into the central hollow and will further displace the metal in the mold, causing its outer sides to rise 80 still higher with the result that as the filling proceeds the rising metal will come into contact with the mold cover and will be caused by the latter to flow inwardly and be turned over on itself into the central space 85 as shown in Fig. 3. As the solidification of the molten mass proceeds from the bottom upwardly, and from the sides inwardly, the central space will become gradually filled from the top supply being poured in, until 90 the mold space is completely occupied by the metal as shown in Fig. 4. The supply of metal may be continued until it backs up in the pouring spout as at 13, thus producing a feeding "head" which will act to 95 maintain the mold completely filled during the final stage of solidification, and will prevent the formation of shrinkage cavities.

As a result of the foregoing operation a sound casting will be produced which will be solid throughout its longitudinal and transverse extent and which will be entirely free from "pipes," shrinkage cavities and like defects.

Having thus described my invention what I claim is:

1. The method of casting ingots, which consists in rotating a mold containing molten metal to cause the same to flow to the outer sides of the mold and rise therein 110 and thereby form a hollow in the body of the metal, supplying molten metal to the

mold and into said hollow to cause the displaced metal to flow inwardly into the hollow, and continuing the supply until the mold is completely filled.

- 5. 2. The method of casting ingots, which consists in rotating a mold containing molten metal to cause the same to flow to the outer sides of the mold and rise therein and thereby form a hollow in the center of 10 the body, supplying molten metal to said hollow to cause the displaced metal to rise still higher at the sides, offering an obstruction to the further rise of the metal to cause the same to be turned inwardly and flow 15 into said hollow, and continuing the supply of metal until the mold is completely filled.
- 3. The method of casting, which consists in rotating a partially filled mold of molten material, supplying additional molten material to the mold during its rotation, continuing the supply of material until the mold is completely filled and maintaining a "head" of the molten material after the mold is filled, and during solidification of 20 25 the metal in the mold.

4. The method of casting, which consists in rotating a covered, partially filled mold of molten material introducing additional molten material through the cover of the mold during its rotation, and continuing the supply of metal to the mold to cause the metal therein to flow against the cover and be deflected thereby toward the center in the body of metal.

5. The method of casting, which consists in rotating a body of molten material about an upright axis situated within the body to cause its sides to rise and form a central hollow, and supplying additional molten material to the central hollow, while causing the rising sides of the body to be turned over onto itself into said hollow, and continuing the supply of metal until the mold is completely filled.

In testimony whereof I have affixed my <sup>45</sup> signature in presence of two witnesses.

HENRY HESS.

Witnesses:

ABRAHAM FELT,  
W. R. KENNEDY.